

# UNITED STATES PATENT OFFICE.

EDWARD D. GLEASON, OF NEW YORK, N. Y., ASSIGNOR TO PLASTIC METAL COMPANY, OF NEW YORK, N. Y., A CORPORATION OF NEW YORK.

## LEAD-COPPER COMPOSITION.

1,077,699.

Specification of Letters Patent.

Patented Nov. 4, 1913.

No Drawing.

Application filed March 7, 1913. Serial No. 752,601.

*To all whom it may concern:*

Be it known that I, EDWARD D. GLEASON, a citizen of the United States, residing in Brooklyn, in the county of Kings, city and 5 State of New York, have invented a certain new and useful Improvement in Lead-Copper Compositions, whereof the following is a specification.

My invention relates to plastic compositions including lead and copper, and lead-copper and tin, which may be advantageously used in the manufacture of bearings for shafts, etc.

It is an object of my invention to provide 15 such compositions free from "lead sweats" and segregation, which are defects usually found in such compositions due to lack of affinity of the lead for the copper or copper and tin, and the high specific gravity and 20 low melting point of lead, for, at best, such compositions are but mechanical mixtures wherein copper is held in a finely divided state in a matrix of lead.

Another object of my invention is to provide 25 such compositions including a given percentage of copper but of different degrees of hardness.

The effect of my improvement is to provide 30 a composition which is homogeneous in that the copper therein is comminuted to the greatest possible extent and equally distributed throughout the mass of the composition. I have discovered that the effect aforesaid is attained by adding to the molten 35 copper, in the process of making such a non-metallic derivative capable of increasing the miscibility of lead and copper, to wit, lead sulfid, and particularly the native lead sulfid, galena. I find it convenient to employ compositions containing lead, lead sulfid, and 40 50 to 60 per cent. copper. For instance, I fuse 50 pounds of copper and add thereto 5 pounds of galena and then gradually add, to said mixture, 45 pounds of lead. The fused 45 mixture is then poured into pig, ingot or other suitable molds, and, when congealed, fracture thereof shows that the cast metal is homogeneous.

Harder compositions may be formed by

taking 50 pounds of copper, 10 pounds of 50 galena and 40 pounds of lead or 45 pounds of copper, 10 pounds of galena and 45 pounds of lead; said ingredients being mixed as in the first instance above described.

As above indicated, the use of galena is effective for the purpose described when used in compositions containing tin. For instance, I take 60 parts copper, 30 parts lead, 5 parts galena and 5 parts tin, or, 55 parts 60 copper, 35 parts lead, 5 parts galena and 5 parts tin. However, such compositions including tin form the subject matter of my application Serial No. 752,600, filed March 7, 1913, for Letters Patent of the United 65 States. Moreover, the process herein contemplated, including the step in the process of alloying copper with another metal which consists in fusing with the copper a non-metallic derivative of the other metal, before 70 mixing the other metal therewith, forms the subject matter of my application Serial No. 757,860 filed March 31, 1913, for Letters Patent of the United States.

Although I have specified compositions 75 containing 50 to 60 per cent. copper, as typical of my invention, I do not desire to limit myself to the precise methods of procedure or proportions herein set forth as it is obvious that various modifications may be 80 made therein without departing from my invention as defined in the appended claims.

I claim:—

1. A composition containing lead, copper, and lead sulfid.
2. A composition containing lead, lead sulfid, and 50 to 60 per cent. copper.
3. A composition containing lead, a non-metallic derivative of lead capable of increasing the miscibility of lead and copper, and copper.

In testimony whereof, I have hereunto signed my name at Philadelphia, Pennsylvania, this sixth day of March, 1913.

EDWARD D. GLEASON.

Witnesses:

ARTHUR E. PAIGE,  
JOHN DOSCHER.

Correction in Letters Patent No. 1,077,699.

It is hereby certified that in Letters Patent No. 1,077,699, granted November 4, 1913, upon the application of Edward D. Gleason, of New York, N. Y., for an improvement in "Lead-Copper Compositions," an error appears in the printed specification requiring correction as follows: Line 35, after the word "such" insert the word *compositions*; and that the said Letters Patent should be read with this correction therein that the same may conform to the record of the case in the Patent Office.

Signed and sealed this 18th day of November, A. D., 1913.

[SEAL.]

R. T. FRAZIER,  
*Acting Commissioner of Patents.*